

Dec. 5, 1944.

W. A. DARRAH

2,364,195

PROCESS OF MAGNESIUM PRODUCTION AND FURNACE EQUIPMENT THEREFOR

Filed June 22, 1942

3 Sheets-Sheet 1



*Fig I*

*Inventor:*

*William A. Darrah*

Dec. 5, 1944.

W. A. DARRAH

2,364,195

PROCESS OF MAGNESIUM PRODUCTION AND FURNACE EQUIPMENT THEREFOR

Filed June 22, 1942

3 Sheets-Sheet 2



Fig. II.

Inventor.

William A. Darrah

Dec. 5, 1944.

W. A. DARRAH

2,364,195

## PROCESS OF MAGNESIUM PRODUCTION AND FURNACE EQUIPMENT THEREFOR

Filed June 22, 1942

3 Sheets-Sheet 3



Fig III.



Fig. IV.

*Inventor:*

William A. Darrah.

## UNITED STATES PATENT OFFICE

2,364,195

PROCESS OF MAGNESIUM PRODUCTION  
AND FURNACE EQUIPMENT THEREFOR

William Austin Darrah, Chicago, Ill.

Application June 22, 1942, Serial No. 447,884

4 Claims. (Cl. 75—10)

This invention relates to a process for preparing metallic magnesium and to electrically heated furnaces designed to operate at pressures below the atmosphere and in a confined space from which air is excluded.

The process and equipment may obviously be applied to numerous other heating and distillation problems such for example as the electro-thermal reduction of zinc, arsenic, and numerous other materials.

The description of the process and equipment will be directed primarily to the reduction of metallic magnesium in order to simply illustrate the principles involved.

Some of the objects of this invention are to economically and rapidly produce large quantities of the metallic magnesium. Other objects are to provide continuous or semi-continuous processes for carrying on this operation.

The process and equipment offered has substantially new advantages in that maintenance which is now a substantial factor in magnesium production is largely eliminated, operating costs are reduced, the heat required is delivered at the required point and not transmitted through an alloy shell. Numerous other objects and advantages will be apparent from a study of the disclosure, drawings and claims submitted herewith.

Referring to the drawings,

Figure I shows in diagram an end elevation of a typical assembly illustrating one form of my invention arranged for continuous operation.

Figure II is a section in plan on the line II—II showing one form of my device.

Figure III is a schematic diagram of one form of arrangement of electric circuits and auxiliaries which contribute to the successful operation of the process and equipment.

Figure IV is an alternate circuit diagram.

Referring to Figure I, reference 1 indicates the furnace equipment used in this process. The furnace equipment is supported on a framework 2 which carries at its upper end a charge hopper 3 connected to furnace chamber 1 by means of duct member 4 provided with tightly closing valves or locks 5 and 6.

At the bottom of furnace member 1 is a similar duct member 7 also provided with tightly closing locks 8 and 9. Hopper 3 is designed to store the charge for feeding to the furnace and discharge duct 7 is designed to provide means of drawing off the ash, clinker or waste from the process.

A duct 10 connects with the furnace at some

convenient point and is designed to provide an exit for the volatile materials liberated by the thermal reaction within the furnace. 11 indicates a cooling chamber provided with an air jacket 12 which is designed to permit maintaining the required temperature in the condenser. Air (or water) is circulated through air jacket 12 entering by inlet 13 and passing through blast gate 14 which is arranged to control the rate of flow of air so that the temperature in the receiving chamber will be sufficient to condense the vapors from the furnace but preferably maintain them in a liquid form. Receiving chamber 11 may be either an empty chamber and the condensate allowed to flow down the inner walls into the discharge hopper 15 at the bottom or as an alternate construction a rotating scraper 16 may be mounted in bearings 17 and 18 and driven by means of motor 19 and V-belt 20 so as to revolve continuously and clean the walls. A housing 21 is indicated as surrounding bearings and motor, to prevent the entrance of air into the rotating system.

If the rotating member 16 is employed it is presumed that the condensate will be collected as a solid dust or powder instead of a liquid although of course the rotary wiper may be utilized in either case.

The rotary wiper may be constructed in any of the known commercial types but is illustrated as comprising a series of arms as for example 22 which carry a scraper bar 23 which revolves in close contact with the inner wall of the condenser 11.

A duct 24 at the bottom of the hopper serves as a lock and members 25 and 26 serve to tightly seal the lock from the atmosphere and from the receiver thus making it possible to remove controlled quantities of the product in the receiver as desired.

Figure II shows in plan more details of the furnace design itself.

In Figure II, 1 indicates the furnace which is enclosed in an air tight steel shell 27 which for convenience may be cylindrical.

Shell 27 is provided with air tight ends 28 and 29 which mount water cooled housings 30 and 31 respectively. Shell 27 is lined with a layer of insulation indicated by 32 and may be provided with an inner layer of insulating refractory 33 and a final layer of magnesite or other highly refractory inert material as indicated by 34. A pair of conducting electrodes 35 and 36 are provided entering the shell through water cooled seal members 38 and 39. These electrodes

may to advantage be formed from graphite or other forms of carbon but I do not wish to be restricted to this material only as numerous other high melting conductors may be employed.

The water cooled seal members 30 and 31 are provided with cooling coils 37 and 38 which carry away the heat conducted through the electrodes and the walls. The space between the electrode and the housing may be filled with an insulating plastic such as tar or bitumin indicated by 39. Bushings of soapstone or porcelain 40 and 41 are provided to insulate the electrode from the steel housing. Internal bushings 42 and 43 are provided to guide and support the electrodes in the hot zone.

Each main power electrode is provided with an ignition electrode indicated by numbers 44 and 45. These electrodes are also sealed into a water cooled housing member 46 and 47, the construction of which is substantially identical, except for size, with the construction of the seal members used on the large electrodes. These seal members are provided with water cooling coils 48 and 49, sealing compounds 50 and 51 and bushings 52 and 53 all as previously described in the case of the larger electrodes.

It will be noted the lining extends around the entire interior of the furnace chamber and for a portion of the duct leading to the receiving chamber. It is desired to reduce the area of the duct as much as possible in order to avoid the loss of radiant heat from the furnace.

54 indicates a thermocouple or other temperature registering device which serves through a standard commercial relay (not shown) to control the delivery of heat to the furnace.

55 indicates a duct or port through the insulating lining connecting to a pipe 56 and an electrically operated valve 57. Valve 57 is connected by pipe 58 to storage chamber 59 containing hydrogen or other inert gases. The object of the assembly including automatic control valve 57 and reservoir 59 is to deliver controlled amounts of gas into the furnace as required by operating conditions.

Referring to Figure III, which shows a diagrammatic arrangement of the electrical circuits used, 1 indicates the furnace, and corresponding parts in the other figures are given corresponding numbers.

60 indicates the secondary or high voltage side of a small high voltage ignition transformer of which 61 is the primary or low voltage side. References 62 and 63 designate a similar transformer.

These transformers are designed to supply a voltage as for example 10,000 volts and are of a construction similar to those used on neon lights, etc. These transformers serve to cause a high voltage discharge which locally heats and ionizes the main power electrodes to permit the arc to start, between 35 and 36.

63A represents the secondary of the main power transformer and 64 represents the primary of the transformer provided with a series of taps as indicated by reference 65.

An excess variable inductance 66 is shown connected into the circuit so as to stabilize the arc formed. 67 indicates one winding of a series transformer of which 68 is the other winding. The series transformer serves by means of a relay 69 to actuate solenoid valve 57 thus allowing gas to enter furnace chamber 1 from the reservoir 59 as required. A short circuiting switch 70 is provided around winding 67 of the

series transformers to cut it out of the circuit when not desired.

The method of operation of the device employed in my process consists in applying a high voltage to the gap between the ignition electrodes and the main power electrodes. This causes a small arc to pass across this gap which locally heats the main power electrodes causing them to reach extremely high local temperature thus causing a flow of electrons from the hot spots and getting them in readiness to support an arc. During this period of the operation the pressure within the furnace chamber should be maintained at a figure substantially below the atmosphere ranging preferably between 26" and 28" absolute of mercury. This may be obtained by means of pump 71 connected to pipe 56 through valve 72.

Having now prepared the power electrodes by localized heating so that they are ready to support an arc power may be applied to the primary 64 of the main power transformer. A current will now flow between electrodes 35 and 36. The flow of current will prove to be somewhat unstable as the arc formed under these conditions will tend to show a lower resistance with an increased current.

This condition may be stabilized by means of the variable inductance 66 or its electrical equivalent, impedance or resistance.

It will be obvious that any of the well known devices for maintaining a substantially constant current in an unstable circuit may be employed. These well known standard devices include such items as the floating coil transformers, formerly used on series arc lighting circuits, the well known induction regulator, and the mere use of a high inductance in series with the power transformer. Transformers having a higher degree of magnetic leakage are quite desirable for this application.

81 and 82 are relays of standard commercial types which are placed so that they operate when the current flowing through the main arc reaches a predetermined value. In other words they are the equivalent of series relays actuated by a minimum current flow in the main circuit. They serve to open the circuit of transformers 62 and 60 which supply power for the auxiliary arc used in starting the main arc.

It will therefore be apparent that these relays provide a means whereby the igniting arcs may be cut out as soon as the main arc is established.

55 Other obvious electrical equivalents may be of course employed to accomplish this same result, the important point being that the auxiliary arc is extinguished when current is passing through the main arc.

60 It will be apparent also with this circuit that if for any reason the main arc is extinguished relays will promptly close the circuits feeding the auxiliary arcs and thus re-establish the circuit between the main electrodes.

65 Figure IV shows an alternate method of starting the main arc initially. This method utilizes the high frequency high voltage ignition circuit. Similar numbers designate similar portions of the equipment.

70 In Figure IV 35 and 36 indicate the main electrodes sealed in an air tight manner into container 1. A source of power, preferably alternating current, at perhaps 1000 volts is applied between the terminals V. Adjustable in-

ductances 88 and 89 are provided in the circuit between the source of power and the electrodes 35 and 36.

Choke coils 92 and 93 are provided in the circuit between the power source and the main electrodes. These choke coils should be designed and insulated to provide an extremely high impedance to high frequency circuits but with a negligible impedance to ordinary commercial power circuits as for example those of 60 cycle frequency.

Connected also to main electrodes 35 and 36 are terminals of a high frequency circuit which will be described. H indicates the terminals of a high frequency circuit which may be obtained from an oscillating spark or arc, from a high frequency generator, vacuum tube oscillator or any similar device, the essential point being that the frequency will be high and the power sufficient to start an arc between electrode 35 and 36.

As an illustration of a practical frequency but one to which I do not wish to be limited I might mention 500,000 cycles per second. Much higher frequencies are satisfactory and in some cases preferable.

94 indicates the primary of a high frequency transformer and 95 a secondary. 96 and 97 indicate capacities or condensers which should be so proportioned in connection with the combined impedance of the transformer formed from coils 94 and 95 that the total impedance of the high frequency circuit feeding electrodes 35 and 36 will be very low and therefore large high frequency current may flow between electrodes 35 and 36 when high frequency power is applied on terminals H.

Other obvious means of providing a high frequency source to cause a discharge between electrodes 35 and 36 are of course well known and may be used.

One of the objects which I am endeavoring to obtain by the circuit disclosed in Figure IV is to provide for "ignition" or starting a high frequency high voltage discharge between electrodes 35 and 36 and arrange the circuit in such a manner that the 60 cycle or other commercial frequency circuit which supplies the main power will sustain the arc once it is started by the high frequency circuit.

It will be apparent that ordinary commercial frequencies provide a much less expensive source of power than high frequency circuits but it is simpler to momentarily start the arc by a high voltage from frequency circuit with a limited amount of power available.

The choke coils 92 and 93 prevent the high frequency high voltage current from passing into the power circuit and also prevent the low impedance of the power circuit (at 60 cycles) from diverting current which is required to pass across the arc.

The condensers 96 and 97 serve to reduce the amount of power from the 60 cycle circuit passing into the high frequency circuit to negligible proportions.

It will of course be evident that while the drawings show a symmetrical arrangement of chokes and condensers, innumerable other circuits accomplishing similar results will be familiar to those skilled in this art.

It is of interest to consider that the production of heat commercially in operations of this type at relatively low pressures by means of an electric arc is a relatively new development and

one which involves new factors not found in present arc furnaces.

Because of the fact that the pressures are very low and that atmospheric oxygen must be eliminated in all gases it is undesirable to have movable electrodes as in the case of most arc furnaces in use today. Since the electrodes are relatively fixed and difficult to move, it then becomes advisable to provide means for starting the arc without moving the electrodes and for adjusting the arc conditions for varying pressures, temperatures, and other factors without moving the electrodes. The accomplishment of these results is part of the object of the equipment and process here disclosed.

At extremely low pressures it is relatively difficult to maintain a stable arc and for this reason provision is made by automatic valve 37 to permit the control and introduction of special gaseous atmospheres. The gas to be introduced depends on the materials being treated and the process. The gases which are to be preferred are the so-called inert gases such as neon, argon, krypton or xenon. In some cases hydrogen may be used. Nitrogen is objectionable in dealing with magnesium because of its tendency to combine with this material. When the current through transformer 68 falls to a predetermined value the relay automatically opens, allowing the inert gas to enter through 38.

Of course oxygen or any gases containing oxygen are quite objectionable as they will react with the magnesium vapor.

Gases containing carbon compounds tend to produce a metallic magnesium seriously contaminated with carbon just as gases containing traces of oxygen produce a metal contaminated with oxide.

The arc at the low pressures employed is quite different from the arc encountered at ordinary atmospheric pressure. At low pressures the arc is "soft" and expands to cover large volumes. The familiar incandescent spots on the surface of the electrodes are also expanded to cover relatively large surfaces.

This condition lends itself peculiarly well to heating applications of the type in question because intense localized heat is avoided but high temperatures can of course be obtained by balancing the heat input against the heat consumption so that there is a continual slight excess.

Localized high temperatures are eliminated.

As an illustration of conditions when operating at pressures somewhere around 29" of mercury, on the barometer column, a voltage of 80 volts across the arc give an arc of around 4" in length with a current flow of around 25 amps.

This is based on carbon electrodes, 60 cycle current, and having an impedance in series with the arc which consumes about 30 volts. Such an arc is extremely stable which is somewhat contrary to conditions ordinarily encountered at atmospheric pressures.

These conditions are mentioned to illustrate the difference between the arc at these low pressures and the arc which would be obtained at normal atmospheric pressures.

The drop across the arc will vary with the nature of the gas or vapor through which the arc is passing, the temperature in the furnace, and to some extent on the configuration of the interior of the furnace. In general the drop between the electrodes appears to be made up of a surface resistance amounting to 10 or 15 volts at

each electrode and appearing within a millimeter or less of the electrode.

The balance of the drop is at the rate of from 5 to 10 volts per inch of arc length subject to much variation with conditions as outlined above.

The radiation from the arc itself is relatively small compared with the radiation encountered at atmospheric pressures. The arc appears to be able to act as a convection heating medium and material emersed in the arc is heated somewhat in the manner that it would be heated if emersed in a salt bath.

Of course some of the important advantages of the low pressures aside from the special facility for arc heating are the ease of causing such reactions as the reduction of magnesium oxides by ferro-silicon or carbon. This is assisted by the higher effective vapor pressure of Si under these conditions.

In the manufacture of metallic magnesium I have found that it is of decided advantage to use a magnesite or a dolemite which is "soft burned" rather than fused and sintered. I attribute this advantage, which shows itself by rapid reactions at lower temperatures and more complete recovery, to the greater facility with which the silicon vapor can contact all portions of the mass to be reacted.

I have found that in producing metallic magnesium it is convenient to utilize briquettes which may be pressed into form and composed of the calcined magnesium oxide (or calcined dolemite) intimately mixed with finely ground silicon or ferro-silicon. The low pressure of course makes it feasible to remove the metallic magnesium produced by evaporation so that the metal is carried out from the briquette as a vapor.

Of course the arc during this portion of the reaction is sustained by the ionization of the magnesium vapor. In other words it is a magnesium arc quite largely.

I prefer to grind the magnesium oxide or dolemite and the reducing agent quite finely. It is desirable to have both materials ground finer than 200 mesh although I am able to carry out the reaction with very much coarser particles.

I have found that briquettes which are somewhat porous give a much quicker reaction, and therefore a greater production per furnace, than briquettes which are dense. Thus I have used sodium silicate as a binder for briquettes and find it less desirable than a binder such as starch.

It is of course evident that in any case the briquettes must be thoroughly dehydrated so that no water is present when they are placed in the furnace.

It is of importance to understand that the equipment here disclosed operates under substantially different conditions from present commercial equipment and the results are different.

Before applying power to the unit it is customary to introduce a charge of material to be heated.

The material may consist of any of the well known substances but one of the most desirable materials are briquettes formed of finely ground intimately mixed powders of magnesite and ferro-silicon or dolemite and ferro-silicon.

Pure metallic silicon finely ground and mixed with magnesite is one of the most desirable materials available to my present knowledge, but this is costly and for commercial operations dolemite and ferro-silicon will give satisfactory re-

sults leaving of course an ash consisting of the iron, silica, calcium oxide, etc.

Of course it is desirable to thoroughly calcine and dehydrate the carbonates of magnesium which are used and I prefer to carry on the calcining at a relatively low temperature and with a long time in order to produce a product having a relatively open structure which accelerates the reaction. This is in distinction to a thoroughly sintered dense structure which appears to retard the reaction.

Instead of using briquettes or other mixtures containing ferro-silicon and magnesium oxide I may use mixtures of magnesium oxide with carbon in which case it is necessary to quickly cool the resultant vapors to prevent a reversible reaction which would reform magnesium from the reduced metal vapor.

Another process which may be carried out in the equipment here disclosed is the vaporization of a mixture of metallic magnesium, oil, carbon, and various other impurities. This mixture may be distilled in the equipment I have disclosed thus setting free metallic magnesium and leaving the carbon and mineral impurities as a residue.

When heat is applied by the arc in air at low pressure the heat will be radiated to the inner sides of the furnace and will raise the temperature of the adjacent briquettes or mixtures so that the reaction between the reducing agent and the magnesia will begin. This will in the case of ferro-silicon and magnesia produce vapors of metallic magnesium which will soon build up pressure within the furnace chamber so that the arc is carried largely by the vapors of metallic magnesium. The magnetic valve and reservoir of hydrogen will only be needed on occasion where the pressure within the chamber becomes so low that it is difficult to quickly heat up the interior of the furnace.

I have found that the flow of current between the electrodes 35 and 36 will vary with several factors and these characteristics must be considered in the design and operation of my equipment. The voltage drop between the electrodes will depend on a constant figure which appears to range from 20 to 30 volts and is dependent largely upon the pressure within the furnace chamber and the nature of the vapor or gas which fills it.

Aside from a somewhat constant voltage drop at the electrodes there will be another consumption of voltage which is proportional to the distance between the ends of the electrodes, that is to say the length of the path of the current flow. This voltage will vary with the pressure of the vapor or gas within the chamber, the nature of the vapor or gas, and the amount of current passing. Values ranging between 2 volts and 20 volts per inch have been found under commercial conditions when operating at effective temperatures and with commercial loads.

When operating steadily at normal temperatures and delivering heat to produce metallic magnesium at a rate of 200 or 300 pounds per hour the voltage will range from 500 to 1000 volts and the current will of course depend on the thermal work to be done and the heat which is lost by radiation.

Normal moderately sized units of the type illustrated will radiate sufficient heat to the atmosphere to maintain the refractories at a safe temperature to give long life and yet a high thermal efficiency.

Large units having of course a relatively smaller

ratio of surface to volume will require additional cooling means such as water pads or water jackets. These are details of construction not essential to the basic invention which I have made.

In order to obtain the maximum production from a given piece of equipment I have found it an advantage as specified previously to utilize a form of magnesium oxide which is as porous and susceptible to reaction as possible. I have found that the best method of producing such a type of oxide is to reduce the carbonates at a low temperature so low that sintering does not occur. This ordinarily gives an oxide which has many of the characteristics of the so-called "caustic burned" oxides.

I have found that by using material of this kind, it is possible to greatly accelerate the reaction and to have a higher recovery of metal and less waste of unreduced oxide.

Obviously the reaction will take place with fused or sintered oxides but ordinarily with lower rates of recovery and higher temperatures and depreciation of the equipment.

One factor which controls the tendency to sinter is the amount of fusible materials or fluxes present in the carbonate. Thus large appreciable amounts of alkali metals, iron, and the various materials which lower the fusion point of the oxide are likely to be detrimental in that they cause sintering at lower temperatures. I therefore prefer to calcine carbonates wherever possible at temperatures and rates such that fusing or sintering of the oxide with the residual impurities will be a minimum.

Having produced a porous and reactive oxide I find that the reduction can be caused to proceed at a still more rapid rate by adding materials which raise the vapor pressure of one or both of the reacting materials. For want of a better term I am calling these "catalysts."

Chlorides represent one class of material which is helpful in this respect and I prefer to use small amounts of magnesium chloride which may be added to the briquettes. Naturally the anhydrous product is to be preferred.

I prefer magnesium chloride to sodium chloride for the reason that the sodium chloride has a tendency to clog the pores of the oxide and thus in some measure retards the reaction.

It is my theory that under the influence of the high temperatures silicon chlorides are formed and these materials are very volatile thus serving as carriers for bringing the silicon into contact with the magnesium oxide.

I do not wish to be confined to any particular compound as many will be recognized as raising the vapor pressure of the metallic silicon or its compounds. In the claims I class this material under the broad heading of a "catalyst."

Having now fully described my invention, what I claim as new and desire to secure by Letters Patent in the United States is:

1. The continuous process of producing magnesium which consists in removing the carbon dioxide from magnesium carbonates at a temperature such that the resultant oxide is relatively porous, mixing said calcined carbonate with non-carbonaceous reducing agent and subjecting the mixture under conditions of low pressure to the direct heat radiated from an electric discharge in low pressure magnesium vapors, to the upper outside surface of said mixture.

2. The process of producing magnesium which consists in removing carbondioxide from magnesium carbonates at a temperature such that the resultant oxide is relatively porous, mixing said calcined carbonate with a carbon-free reducing agent and subjecting the upper surface of said mixture under conditions of low pressure to the heat directly radiated from an electric discharge in magnesium vapors.

3. In the process of producing magnesium, the steps of producing a porous active non-sintered oxide of magnesium, mixing said oxide while in said active state with a noncarbonaceous material containing elemental silicon and heating the upper surface of said mixture under conditions of low pressure by passing an electric current through the vapor of the metal being reduced, and causing the direct radiation of said electric arc to radiate to said mixture, thus heating the upper surface of said mixture to a higher temperature than the balance of the mixture.

4. In the process of producing metallic magnesium the step of heating a mixture containing magnesium oxide with a noncarbonaceous reducing agent under conditions of low pressure, by means of direct radiation from an electric discharge supported by magnesium vapor at low pressure, said radiation directly heating the upper surface of said mixture initially to a higher temperature than the balance of said mixture so that the reaction first takes place in the upper surface which results in the evolution of magnesium vapor from the upper surface under such conditions that the bulk of the vapor does not travel through the entire mass of the mixture.